# EUROPEAN PATENT SPECIFICATION

(11) **EP 1 409 756 B1**
(45) Date of publication and mention of the grant of the patent: **20.09.2006**
(21) Application number: 02743117.0
(22) Date of filing: 28.05.2002
(51) Int. Cl.: C22C 19/05, C22C 38/44, C23F 13/00

(54) **STEEL PARTS MADE OF AUSTENITIC OR SEMI-AUSTENITIC STEEL IN A PLANT FOR PRODUCING SULFURIC ACID AND METHOD FOR THE PROTECTION AGAINST CORROSION**
AUS AUSTENITISCHEM ODER HALBAUSTENITISCHEM STAHL BESTEHENDE TEILE EINER ANLAGE ZUR HERSTELLUNG VON SCHWEFELSÄURE UND VERFAHREN ZUM KORROSIONSCHUTZ
PIECES EN ACIER AUSTENITIQUE OU SEMI-AUSTENITIQUE DANS UNE INSTALLATION DE PRODUCTION D'ACIDE SULFURIQUE ET PROCEDE DE PROTECTION CONTRE LA CORROSION

(30) Priority: 08.06.2001 DE 10128032
(43) Date of publication of application: 21.04.2004
(73) Proprietor: Outokumpu Technology Oy, 02200 Espoo (FI)
(72) Inventor: DAUM, Karl-Heinz, 55124 Mainz (DE); RAUSER, Wolf-Christopf, Wembley Downs 6019 WA (AU); ANASTASIJEVIC, Nikola, 63674 Altenstadt (DE); SCHALK, Wolfram, 61267 Neu-Anspach (DE); LAIBACH, Stefan, 36419 Geismar/Rhön (DE); SCHNAUBELT, Herbert, 61184 Karben (DE)
(74) Representative: KEIL & SCHAAFHAUSEN Patentanwälte
(86) International application number: PCT/EP2002/005842
(87) International publication number: WO 2002/101106

(56) References cited:
- EP-A- 0 018 124
- EP-A- 0 130 967
- EP-A- 0 937 680
- US-A- 4 588 022
- US-A- 5 028 396
- US-A- 5 695 716

## Description

This invention relates to a method for the protection against corrosion of steel parts made of austenitic or semi-austenitic steel during the production of sulfuric acid and to respective steel parts.

In general, sulfuric acid is produced by the catalytic conversion of the SO₂ content of gases to obtain SO₃ and - in the case of dry gases - by the subsequent absorption of the SO₃ formed in concentrated sulfuric acid or - in the case of humid gases - by the subsequent condensation of the sulfuric acid formed. The usual technical components such as drier, absorber, heat exchanger etc. get in contact with concentrated sulfuric acid starting at about 93 wt-% and an elevated temperature. This sulfuric acid is extremely aggressive and exerts a fast and strong corrosion on the structural parts to be used. Therefore, the structural parts which get in contact with sulfuric acid must be made of corrosion-resistant materials. Special ferritic steel alloys, cast iron, plastics, ceramics, glass or other materials with a corresponding lining turned out to be particularly corrosion-resistant. For these applications, the non-metallic materials generally have unfavorable mechanical properties and are difficult to process. The metallic materials have good mechanical properties, but their corrosion resistance is not sufficient, or the materials are very expensive. In particular for use in heat exchangers, very thin-walled components are required, which need a high transfer of heat. In these components, the previous corrosion resistance no longer is sufficient. These plants are usually operated with a sulfuric acid concentration ≥ 93 wt-% to 100 wt-% and a temperature up to 140°C. A known method of corrosion protection is the anodic corrosion protection. In this method, the materials to be protected are coated with a metal oxide layer which prevents the corrosion attack.

The use of austenitic steels during the production of sulfuric acid is known from EP 0 130 967. The steel grades indicated in this protective right are intended in particular for use in heat exchangers. The materials used here do not satisfy the requirements which must now be fulfilled by corrosion-resistant materials. For the technical plants now in use smaller corrosion rates are required in particular.

In order to improve the corrosion resistance, US 5,028,396 proposes austenitic stainless steels with a relatively high silicon content consisting essentially of 17.5 % Cr, 17.5 % Ni, 4.6 to 5.8 % Si, the balance being Fe.

Furthermore, US 5,695,716 discloses austenitic, corrosion resistant chromium, nickel iron alloys including at least 32 wt-% chromium.

DE 38 30 365 describes the use of ferritic chromium-molybdenum steels which are resistant to sulfuric acid with a concentration from 94 wt-% onwards and with a temperature below the boiling point. These ferritic steels are very expensive and more difficult to process than austenitic steels. The corrosion resistance is not regarded as sufficient either.

Proceeding from this prior art, it is the object underlying the invention to improve the protection against corrosion of at least one steel part of a device made of austenitic or semi-austenitic steel during the production of sulfuric acid, in which device the steel part gets in contact with the sulfuric acid.

In accordance with the invention, there is provided a method comprising the features of claim 1.

Advantageous embodiments of the invention are evident from the dependent claims.

Experiments have shown that steel grades with a Cr content of 15 wt-% to 26.2 wt-%, a Ni content of 9 wt-% to 25.2 wt-% and a Si content of 0.75 wt-% at most are particularly resistant to corrosion.

In terms of corrosion resistance, especially the elements silicon and chromium from among the chemical alloying elements are known to form a passive layer, whereas the chemical elements nickel and molybdenum weaken the formation of a passive layer,

The ratio of the chemical elements (Cr + Si)/(Ni + Mo) in the range from 1.01 to 1.34 turned out to be particularly advantageous.

Likewise, for those steel grades which only have a minor content of silicon there was obtained an advantageous ratio of the chemical elements Cr/(Ni + Mo) in the range from 0.8 to 1.1.

The ratio is particularly favorable when molybdenum is present in a not too large amount of 0 wt-% to 2.5 wt-%. Depending on the availability of the steel grades to be supplied for the raw materials such as tubes or sheets, austenitic or semi-austenitic steel parts with a molybdenum content of 2 wt-% to 2.5 wt-% can be used.

What is particularly critical for corrosion are those ranges in which the concentration of sulfuric acid is about 97 wt-% to 99 wt-% or the temperature of sulfuric acid is about 160°C to 230°C.

During the production of sulfuric acid, components particularly susceptible to corrosion are heat exchangers, such as e.g. plate-type heat exchangers or shell-and-tube heat exchangers, as well as the entire pipe system.

Embodiments of the process will be explained by way of example with reference to the drawing, in which:
- Fig. 1: shows the current density/potential curve of an austenitic material,
- Fig. 2: is a schematic representation of the anodic protection in a heat exchanger.

Fig. 1 shows the current density/potential curve of a typical austenitic material containing 16.5 to 18.5 wt-% chromium, 11 to 14 wt-% nickel and 2 to 2.5 wt-% molybdenum. In this measurement, sulfuric acid was used as medium with 98 wt-% at a temperature of 200°C. As cathode, there was used a steel cathode made of 1.4404. On the abscissa, the potential is plotted in millivolt (mV) against a Hg/HgSO₄ reference electrode, and on the ordinate the current density is plotted in milliampere per square centimeter (mA/cm²). There can also be used other reference electrodes, such as e.g. a calomel electrode or a cadmium bar.

The first part of the diagram in the range from 0 to 600 mV shows a peak which is referred to as active potential. In the range from 600 mV to 1800 mV then follows the saddle of the curve, the so-called passive potential. The subsequent rise from 1800 mV is referred to as transpassive potential. To achieve a corrosion protection as effective as possible in the anodic corrosion protection, the current density must lie within the range of the passive potential. The values represented here are exemplary, as they are material- and temperature-dependent.

Fig. 2 shows the arrangement of the anodic corrosion protection in a shell-and-tube heat exchanger (1) for sulfuric acid. Via a connection (2), cooling medium is introduced into a first chamber (3) of a shell-and-tube heat exchanger (1). From there, the cooling medium is distributed and flows through individual tubes (4) into a second chamber (5), from which the cooling medium is discharged again. By way of example, only two tubes (4) are represented here.

Via a further connection (6), hot sulfuric acid is introduced. The sulfuric acid flows around the tubes (4) filled with cooling medium and is discharged again via the connection (7). When flowing around the tube bundles (4), the sulfuric acid is cooled.

A plurality of metal cathodes (8) are mounted between the tubes (4) in the shell-and-tube heat exchanger. The representation shows a cathode (8) by way of example. The number of cathodes (8) used depends on the size of the heat exchanger and also on the temperature and the concentration of the sulfuric acid. The cathode (8) is made of the material 1.4404 and is in permanent contact with the sulfuric acid. The cathode (8) is connected with the negative pole of a potentiostat (9) by an electric line. The potentiostat (9) is a d.c. voltage source whose positive pole (10) is connected with the parts of the shell-and-tube heat exchanger (1) to be protected via an electric line.

A second reference electrode (11) is inserted in the shell-and-tube heat exchanger via a seal and is connected with the potentiostat (9) via an electric line. This reference electrode (11) likewise is permanently surrounded by the sulfuric acid and provides the measurement basis for the potentiostat (9). By means of the electric voltage between reference electrode (11) and cathode (8), the potential required for the corrosion protection is determined and adjusted at the potentiostat (9).

In the subsequent Table, the corrosion behavior of the materials in accordance with the invention is shown at different temperatures and a sulfuric acid concentration of 98 wt-%. The flow rate of the sulfuric acid was 1 m/s. The corrosion behavior was determined by immersion tests. In all cases, the test period was 7 days. The removal rates were determined by measuring the corrosion flow and by conversion to mm/a. The test medium was renewed after each test cycle.

| | **Temperature [°C]** | **1.4571** | **1.4404** | **1.4465** | **1.4591** |
|---|---|---|---|---|---|
| **Corrosion rate mm/a** | 160 | 0.02 | 0.03 | 0.15 | - |
| | 180 | 0.06 | 0.04 | 0.06 | 0.01 |
| | 200 | 0.04 | 0.10 | 0.14 | 0.11 |

Thus, the corrosion rates are distinctly lower than in the previous prior art.

## Claims

1. A method for the protection against corrosion of at least one steel part of a device which is used in a plant for producing sulfuric acid, and in which the steel part gets in contact with concentrated sulfuric acid, **characterized in that** at a sulfuric acid concentration of 93 wt-% up to 100 wt-% and a temperature of 140°C up to the boiling point of the sulfuric acid, the steel part is made of austenitic or semi-austenitic steel which has a Cr content of 15 wt-% to 26.2 wt-%, a Ni content of 9 wt-% to 25.2 wt-% and a Si content of up to 0.75 wt-%, and in which the ratio of the chemical elements (Cr + Si)/(Ni + Mo) lies in the range from 0.9 to 1.9 or in which the ratio of the chemical elements Cr/(Ni + Mo) lies in the range from 0.8 to 1.5, and in which the steel part has an anodic corrosion protection, wherein an anode, a cathode and a reference electrode are connected with a potentiostat which supplies an adjustable direct electric current, and wherein the cathode and the reference electrode are in contact with the sulfuric acid and the anode is in contact with the steel part.

2. The method as claimed in claim 1, **characterized in that** the ratio of the chemical elements (Cr + Si)/(Ni + Mo) lies in the range from 1.01 to 1,34.

3. The method as claimed in claim 1, **characterized in that** the ratio of the chemical elements Cr/(Ni + Mo) lies in the range from 0,8 to 1.1.

4. The method as claimed in claim 1, **characterized in that** the steel part is made of austenitic or semi-austenitic steel which has a molybdenum content of 0 wt-% to 2.5 wt-%.

5. The method as claimed in claim 1, **characterized in that** the steel part has a molybdenum content of 2 wt-% to 2.5 wt-%.

6. The method as claimed in claim 1, **characterized in that** the steel part is made of steel 1.4465.

7. The method as claimed in claim 1, **characterized in that** the concentration of the sulfuric acid lies in the range from 97 wt-% to 99 wt-%.

8. The method as claimed in claim 1, **characterized in that** the temperature of the sulfuric acid is about 160°C to 230°C.

9. The method as claimed in claim 1, **characterized in that** the steel part is used in a heat exchanger.

10. The method as claimed in claim 1, **characterized in that** the steel part is used in an acid-conducting pipe.

11. A heat exchanger (1) used in a plant for producing sulfuric acid and comprising at least one steel part being in contact with concentrated sulfuric acid having a sulfuric acid concentration of 93 wt-% up to 100 wt-% and a temperature of 140°C up to the boiling point of the sulfuric acid,
wherein the steel part has an anodic corrosion protection, wherein an anode, a cathode (8) and a reference electrode (11) are connected with a potentiostat (9) which supplies an adjustable direct electric current, and wherein the cathode (8) and the reference electrode (11) are in contact with the sulfuric acid and the anode is in contact with the steel part,
wherein the steel part is made of austenitic or semi-austenitic steel,
**characterized in that** the steel has
a Cr content of 15 wt-% to 26.2 wt-%,
a Ni content of 9 wt-% to 25.2 wt-% and
a Si content of up to 0,75 wt-%,
and in which the ratio of the chemical elements (Cr + Si)/(Ni + Mo) lies in the range from 0.9 to 1.9 or
in which the ratio of the chemical elements Cr/(Ni + Mo) lies in the range from 0.8 to 1.5.

12. The heat exchanger as claimed in claim 11, **characterized in that** the steel part is made of steel 1.4465.

13. An acid-conducting pipe used in a plant for producing sulfuric acid and comprising at least one steel part being in contact with concentrated sulfuric acid having a sulfuric acid concentration of 93 wt-% up to 100 wt-% and a temperature of 140°C up to the boiling point of the sulfuric acid,
wherein the steel part has an anodic corrosion protection, wherein an anode, a cathode (8) and a reference electrode (11) are connected with a potentiostat (9) which supplies an adjustable direct electric current, and wherein the cathode (8) and the reference electrode (11) are in contact with the sulfuric acid and the anode is in contact with the steel part,
wherein the steel part is made of austenitic or semi-austenitic steel,
**characterized in that** the steel has
a Cr content of 15 wt-% to 26.2 wt-%,
a Ni content of 9 wt-% to 25.2 wt-% and
a Si content of up to 0.75 wt-%,
and in which the ratio of the chemical elements (Cr + Si)/(Ni + Mo) lies in the range from 0.9 to 1.9 or
in which the ratio of the chemical elements Cr/(Ni + Mo) lies in the range from 0.8 to 1.5.

14. The acid-conducting pipe as claimed in claim 13, **characterized in that** the steel part is made of steel 1.4465.

## Patentansprüche

1. Ein Verfahren zum Schutz gegen Korrosion wenigstens eines Stahlteils einer Vorrichtung, die in einer Anlage zur Herstellung von Schwefelsäure verwendet wird, und bei dem das Stahlteil in Kontakt mit konzentrierter Schwefelsäure kommt, **dadurch gekennzeichnet, dass** bei einer Schwefelsäurekonzentration von 93 Gew.-% bis 100 Gew.-% und einer Temperatur von 140°C bis zum Siedepunkt der Schwefelsäure das Stahlteil aus austenitischem oder halbaustenitischem Stahl besteht, welcher einen Cr-Gehalt von 15 Gew.-% bis 26,2 Gew.-%, einen Ni-Gehalt von 9 Gew.-% bis 25,2 Gew.-% und einen Si-Gehalt von bis zu 0.75 Gew.-% aufweist, und bei dem das Verhältnis der chemischen Elemente (Cr + Si)/(Ni + Mo) im Bereich von 0,9 bis 1,9 liegt oder bei dem das Verhältnis der chemischen Elemente Cr/(Ni + Mo) im Bereich von 0,8 bis 1,5 liegt, und bei dem das Stahlteil einen anodischen Korrosionsschutz aufweist, wobei eine Anode, eine Kathode und eine Bezugselektrode mit einem Potentiostaten verbunden sind, der einen einstellbaren elektrischen Gleichstrom liefert, und wobei die Kathode und die Bezugselektrode mit der Schwefelsäure und die Anode mit dem Stahlteil in Kontakt stehen.

2. Das Verfahren nach Anspruch 1, **dadurch gekennzeichnet, dass** das Verhältnis der chemischen Elemente (Cr + Si)/(Ni + Mo) im Bereich von 1,01 bis 1,34 liegt.

3. Das Verfahren nach Anspruch 1, **dadurch gekennzeichnet, dass** das Verhältnis der chemischen Elemente Cr/(Ni + Mo) im Bereich von 0,8 bis 1,1 liegt.

4. Das Verfahren nach Anspruch 1, **dadurch gekennzeichnet, dass** das Stahlteil aus einem austentischen oder halbaustenitischen Stahl besteht, welcher einem Molybdängehalt von 0 bis 2,5 Gew.-% aufweist.

5. Das Verfahren nach Anspruch 1, **dadurch gekennzeichnet, dass** das Stahlteil einen Molybdängehalt von 2 bis 2,5 Gew.-% hat.

6. Das Verfahren nach Anspruch 1, **dadurch gekennzeichnet, dass** das Stahlteil aus Stahl 1.4465 hergestellt ist.

7. Das Verfahren nach Anspruch 1, **dadurch gekennzeichnet, dass** die Konzentration der Schwefelsäure im Bereich von 97 Gew.-% bis 99 Gew.-% liegt.

8. Das Verfahren nach Anspruch 1, **dadurch gekennzeichnet, dass** die Temperatur der Schwefelsäure etwa 160°C bis 230°C beträgt.

9. Das Verfahren nach Anspruch 1, **dadurch gekennzeichnet, dass** das Stahlteil in einem Wärmetauscher verwendet wird.

10. Das Verfahren nach Anspruch 1, **dadurch gekennzeichnet, dass** das Stahlteil in einem Säureleitungsrohr verwendet wird.

11. Ein Wärmetauscher (1), der in einer Anlage zur Herstellung von Schwefelsäure verwendet wird und wenigstens ein Stahlteil aufweist, das in Kontakt mit konzentrierter Schwefelsäure steht, die eine Schwefelsäurekonzentration von 93 Gew.-% bis 100 Gew.-% und eine Temperatur von 140°C bis zu dem Siedepunkt der Schwefelsäure hat,
wobei das Stahlteil einen anodischen Korrosionsschutz aufweist, wobei eine Anode, eine Kathode (8) und eine Bezugselektrode (11) mit einem Potentiostaten verbunden sind, der einen einstellbaren elektrischen Gleichstrom liefert, und
wobei die Kathode (8) und die Bezugselektrode (11) in Kontakt mit der Schwefelsäure und die Anode in Kontakt mit dem Stahlteil stehen,
wobei das Stahlteil aus austenitischem oder halbaustenitischem Stahl besteht,
**dadurch gekennzeichnet, dass** der Stahl
einen Cr-Gehalt 15 Gew.-% bis 26,2 Gew.-%,
einen Ni-Gehalt von 9 Gew.-% bis 25,2 Gew.-% und
einen Si-Gehalt von bis zu 0,75 Gew.-% aufweist,
und bei dem das Verhältnis der chemischen Elemente (Cr + Si)/(Ni + Mo) im Bereich von 0,9 bis 1,9 liegt oder
bei dem das Verhältnis der chemischen Elemente Cr/(Ni + Mo) im dem Bereich von 0,8 bis 1,5 liegt.

12. Der Wärmetauscher nach Anspruch 11, **dadurch gekennzeichnet, dass** das Stahlteil aus Stahl 1.4465 hergestellt ist.

13. Ein Säureleitungsrohr, das in einer Anlage zur Herstellung von Schwefelsäure verwendet wird und wenigstens ein Stahlteil aufweist, das in Kontakt mit konzentrierter Schwefelsäure steht, die eine Schwefelsäurekonzentration von 93 Gew.-% bis 100 Gew.-% und eine Temperatur von 140°C bis zu dem Siedepunkt der Schwefelsäure hat,
wobei das Stahlteil einen anodischen Korrosionsschutz aufweist, wobei eine Anode, eine Kathode (8) und eine Bezugselektrode (11) mit einem Potentiostaten verbunden sind, der einen einstellbaren elektrischen Gleichstrom liefert, und wobei die Kathode (8) und die Bezugselektrode (11) in Kontakt mit der Schwefelsäure und die Anode in Kontakt mit dem Stahlteil stehen,
wobei das Stahlteil aus austenitischem oder halbaustenitischem Stahl besteht,
**dadurch gekennzeichnet, dass** der Stahl
einen Cr-Gehalt 15 Gew.-% bis 26,2 Gew.-%,
einen Ni-Gehalt von 9 Gew.-% bis 25,2 Gew.-% und
einen Si-Gehalt von bis zu 0,75 Gew.-% aufweist,
und bei dem das Verhältnis der chemischen Elemente (Cr + Si)/(Ni + Mo) im Bereich von 0,9 bis 1,9 liegt oder
bei dem das Verhältnis der chemischen Elemente Cr/(Ni + Mo) im dem Bereich von 0,8 bis 1,5 liegt.

14. Das Säureleitungsrohr nach Anspruch 13, **dadurch gekennzeichnet, dass** das Stahlteil aus Stahl 1.4465 hergestellt ist.

## Revendications

1. Procédé pour la protection contre la corrosion au moins d'une partie d'acier d'un mécanisme utilisé dans une installation à produire de l'acide sulfurique, la partie d'acier étant mise contact avec l'acide sulfurique concentré, **caractérisé en ce qu'** à une concentration de l'acide sulfurique dans la partie d'acier entre 93 pourcentage en poids et 100 pourcentage en poids et à une température entre 140°C et le point d'ébullition de l'acide sulfurique, la partie d'acier est formée d'acide austénitique ou demi-austénitique d'une teneur en Cr entre 15 pourcentage en poids et 26,2 pourcentage en poids, d'une teneur en Ni entre 9 pourcentage en poids et 25,2 pourcentage en poids et d'une teneur en Si tout au plus de 0,75 pourcentage en poids, ou la relation des éléments chimiques (Cr + Si) / (Ni + Mo) est entre 0,9 et 1,9 respectivement la relation des éléments chimiques Cr / (Ni + Mo) est entre 0,8 et 1,5, la partie d'acier étant prévue d'une protection anodique contre la corrosion, une anode, une cathode et une électrode de référence étant reliées à un potentiostat délivrant un courant continu ajustable, où la cathode et l'électrode de référence est en contact avec l'acide sulfurique tandis que l'anode est en contact avec la partie d'acier.

2. Procédé selon la revendication 1, **caractérisé en ce que** la relation des éléments chimiques (Cr + Si) / (Ni + Mo) est entre 1,01 et 1,34.

3. Procédé selon la revendication 1, **caractérisé en ce que** la relation des éléments chimiques Cr / (Ni + Mo) est entre 0,8 et 1,1.

4. Procédé selon la revendication 1, **caractérisé en ce que** la partie d'acier est formée d'acier austénitique ou demi-austénitique d'une teneur en molybdène entre 0 et 2,5 pourcentage en poids.

5. Procédé selon la revendication 1, **caractérisé en ce que** la partie d'acier est d'une teneur en molybdène entre 2 et 2,5 pourcentage en poids.

6. Procédé selon la revendication 1, **caractérisé en ce que** la partie d'acier est formée d'acier 1,4465.

7. Procédé selon la revendication 1, **caractérisé en ce que** la concentration de l'acide sulfurique est entre 97 pourcentage en poids et 99 pourcentage en poids.

8. Procédé selon la revendication 1, **caractérisé en ce que** la température de l'acide sulfurique est environ entre 160°C et 230°C.

9. Procédé selon la revendication 1, **caractérisé en ce que** la partie d'acier est utilisée dans un appareil d'échange de chaleur.

10. Procédé selon la revendication 1, **caractérisé en ce** la partie d'acier est utilisée dans un tuyau conduisant de l'acide.

11. Appareil d'échange de chaleur (1) utilisé dans une installation à produire de l'acide sulfurique et comportant au moins une partie d'acier étant en contact avec de l'acide sulfurique concentré d'une concentration entre 93 pourcentage en poids et 100 pourcentage en poids et d'une température entre 140°C et le point d'ébullition de l'acide sulfurique,
la partie d'acier étant prévue d'une protection anodique contre la corrosion, où une anode, une cathode (8) et une électrode en référence (11) sont reliées à un potentiostat (9) délivrant un courant continu ajustable, la cathode (8) et l'électrode en référence étant en contact avec l'acide sulfurique et l'anode étant en contact avec la partie d'acier,
la partie d'acier étant formée d'acier austénitique ou demi-austénitique,
**caractérisé en ce que** l'acier a
une teneur en Cr entre 15 % en poids et 26,2 % en poids,
une teneur en Ni entre 9 % en poids et 25,2 % en poids, et
une teneur en Si tout au plus de 0,75 % en poids
la relation des éléments chimiques (Cr + Si) / (Ni + Mo) étant entre 0,9 et 1,9, et
la relation des éléments chimiques Cr / (Ni + Mo) étant entre 0,8 et 1,5.

12. Appareil d'échange de chaleur selon la revendication 11, **caractérisé en ce que** la partie d'acier est formée d'acier 1.4465.

13. Tuyau conduisant de l'acide utilisé dans une installation à produire de l'acide sulfurique, comportant ou moins une partie d'acier mise en contact avec l'acide sulfurique concentré d'une concentration entre 93 pourcentage en poids et 100 pourcentage en poids, et d'une température entre 140°C et le point d'ébullition de l'acide sulfurique,
la partie d'acier étant prévue d'une protection anodique contre la corrosion, où une anode, une cathode (8) et une électrode en référence (11) sont reliées à un potentiostat (9) délivrant un courant continu ajustable, la cathode (8) et l'électrode en référence étant en contact avec l'acide sulfurique et l'anode étant en contact avec la partie d'acier,
la partie d'acier étant formée d'acier austénitique ou demi-austénitique,
**caractérisé en ce que** l'acier a
une teneur en Cr entre 15 % en poids et 26,2 % en poids,
une teneur en Ni entre 9 % en poids et 25,2 % en poids, et
une teneur en Si tout au plus de 0,75 % en poids
la relation des éléments chimiques (Cr + Si) / (Ni + Mo) étant entre 0,9 et 1,9, et
la relation des éléments chimiques Cr / (Ni + Mo) étant entre 0,8 et 1,5.

14. Le tuyau conduisant de l'acide selon la revendication 13, **caractérisé en ce que** la partie d'acier est formée d'acier 1.4465.
